

## UNITED STATES PATENT OFFICE

2,554,364

## PROCESS OF EXFOLIATING MARINE SHELL PLATELETS

Joseph H. Hooton, Englewood, N. J., assignor to  
Richelieu Corporation, New York, N. Y., a corporation of New York

No Drawing. Application April 9, 1949,  
Serial No. 86,599

5 Claims. (Cl. 252—378)

1

This invention relates to a new and novel process of separating iridescent crystal platelets from marine and fresh water shells.

The beautiful appearance of the nacre or mother-of-pearl material contained in fresh water or marine shells such as the abalone shells, snail shells, pearl oyster shells and other mussel shells is well known and it has often been tried to separate the crystals or platelets in such a condition that they could be employed for imparting a decorative effect to other materials. The decorative portion of these shells is made up of platelets or lamellae of calcium carbonate crystal particles held together by a proteinaceous substance called conchiolin. In separating the crystals by a delamination or exfoliation process all of the protein binder must not be removed or altered because it is apparently the thin coating of this material on the calcium carbonate crystals which gives such crystals their iridescence and shiny appearance. The lamella can be separated by heat alone but this process destroys or changes the conchiolin or protein binder so that only dull, white or gray crystals are obtained.

These shell crystals have attracted the attention of many inventors and many attempts have been made to separate the plate like crystals from each other and from the remainder of the shell. For example, U. S. Patent No. 1,570,183 discloses that the laminae or flakes may be separated by heating the shells. Heat however destroys a considerable portion if not all of the luster of the crystal particles. U. S. Patent No. 1,812,885 discloses a process of exfoliating the shells by heating in the presence of water at relatively high temperature and pressures. U. S. Patent No. 2,172,369 discloses another process of producing such crystals which involves heating the shells in the presence of a mild aqueous alkaline solution. The heat required according to this latter patent is less than that required in the other two patents but nevertheless the shells are eventually subjected to the alkaline solution at a temperature of 100° C. This patent also discloses but does not claim a process of exfoliation at 25° in ammonia solutions but the time required is excessively long. There is evidence to indicate that the iridescent appearance of the crystals in a shell is at least partly due to a thin coating of proteinaceous material on the surface of the crystal particle. Any considerable amount of heat is also known to cause coagulation or denaturation of proteins. If the crystal particles could be separated by processes involving not

2

heating of the crystals there would be less likelihood of damaging the surface coating of the crystals and the resultant products should have increased luster and sparkle.

5 An object of this invention therefore is to provide a process of separating the crystal platelets from shell particles without subjecting the crystal platelets to temperatures of boiling water or any temperature sufficiently high to cause coagulation or denaturation of proteins.

10 Another object of this invention therefore is to provide a process for separating decorative, iridescent, silvery and sparkling crystals from marine and fresh water shells.

15 Another object of the invention is to provide a process of separating the crystal platelets of marine and fresh water shells in substantially the same state as they appear in the shells.

20 Another object of the invention is to provide a method of exfoliating shell material without destroying the proteinaceous coating on the calcium carbonate particles of the shells.

25 Another object of the invention is to provide a method for producing silvery bleached crystal platelets from shells, which platelets retain their natural sparkle and iridescence.

30 These objects and others ancillary thereto are obtained by exfoliating the shells or shell fragments by a mild chemical treatment with an aqueous solution containing a mild alkaline buffer reagent such as an alkali phosphate. Preferably before or during the treatment the shells are subjected to a mechanical or a chemical process to remove the backs or other portions thereof which might produce discolored particles and it is also desirable to grind, cut or crush the shells to fragments of convenient size, for example, to a size of 1.4" to 2 inches on a side. Prior to and/or during exfoliating the shell particles are preferably treated with a bleaching agent to produce a product with more of a silvery aspect. In the last stages of the exfoliating process, especially, the process is carried out without subjecting the particles to high temperatures and preferably without any extraneous heat.

35 The phosphates which may be employed in the exfoliation process include the di- and tri-sodium phosphate ( $Na_2HPO_4$ ) and ( $Na_3PO_4$ ) sodium pyrophosphate ( $Na_4P_2O_7$ ), sodium tri-polyphosphate ( $Na_5P_3O_{10}$ ), the sodium metaphosphates, ( $Na_4PO_3$ ), sodium monothiotetraphosphate ( $Na_6P_4O_{12}S$ ), sodium trithiotetraphosphate ( $Na_6P_4O_{10}S_3$ ) sodium tetraphosphate ( $Na_6P_4O_{13}$ ) mixtures of such phosphates, and the

corresponding potassium, ammonium and lithium compounds.

Alkaline reagents such as ammonium, sodium or potassium carbonates are added to the phosphate solutions to produce a solution which has a pH of 10-13. It is also possible to employ a dilute solution of the alkali hydroxides, without additional phosphates, in the early stages of the exfoliation process but the final exfoliation step should be conducted without heat and in the absence of strong alkalies. The alkali solution should be of less than normal concentration and the product should be thoroughly washed after the treatment. It is preferred to conduct the exfoliation treatment with alkaline solutions at room temperatures but it is possible to heat the alkaline exfoliating solutions to as high as 70° C. without destroying too much of the luster and silvery appearance. The treatment with chlorine water restores the silvery luster and in some cases even increases the silvery appearance to a greater degree than that present in the original shells.

This improved sparkle and silvery luster produced by treatment with the mild oxidizing agents is unpredictable. For such treatments aqueous solutions of chlorine, oxygen, hydrogen peroxide, sodium peroxide and sodium hypochlorite have been found suitable. Bleaching agents, such as potassium permanganate, which impart a color to aqueous solutions do not improve the luster of the product.

It is sometimes desirable to conduct the exfoliation treatment with the alkaline solutions in several stages the most drastic treatment being applied first and to treat with the oxidizing agents between two of the exfoliating stages. In this way the alkalinity of the final exfoliating liquor can be decreased and the total time required for the treatment can also be decreased.

It has also been found that if a very small amount of a fluorescent dye, such as fluorescene, umbelliferone, beta methyl umbelliferone, etc. is added to the exfoliating liquor, an added sparkle and color is obtained in the final product.

The novel features characteristic of this invention are set forth with particularity in the appended claims. The invention itself, however, both as to its organization and its method of operation, together with additional objects and advantages thereof, will best be understood from the following description of specific embodiments when read in connection with the following examples:

*Example 1*

The shells known commercially as Kapiz shells (the scientific name is *Placuna Placenta Linn*) having the unsightly backs removed (as by grinding) are broken into fragments averaging about  $\frac{1}{4}$  to 1 square inch in size.

One hundred pounds of these fragments are then placed in a vessel and covered with a solution of 12½ pounds of trisodium phosphate in 190 pounds of water to which are added 5 pounds of a mixture of the sodium tetraphosphate with the sodium mono and trithiotetra phosphates.

This mixture of shells and liquor is allowed to stand at room temperature for 48 hours during which time the crystals are exfoliated.

The solution is poured off and the separated crystals are washed with cold water until the chemicals from the previous treatment are eliminated. The flat platelets or crystals which separate are about  $\frac{1}{16}$  to  $\frac{1}{4}$  on a side and have a sparkling and iridescent appearance. These crys-

tals are then dried in a current of air which, while the crystals are still damp, may have a temperature as high as 250° F.

*Example 2*

5 Kapiz shells are cleaned and crushed or ground to a size of  $\frac{1}{16}$  to  $\frac{1}{4}$  on a side. The broken shell is treated in 3% hydrochloric acid to remove the discolored porous backs and then washed with 10 ordinary water to remove the remaining acid and soluble salts resulting from the acid treatment.

These shell particles are then placed in a chlorine solution made up as follows:

Water, 48 gallons

15 15% solution of gaseous chlorine, 9 gallons  
Shell particles, 100 pounds

The shell particles are soaked in this solution at room temperature for 2 hours. Then the solution is poured off and the shells are washed with 20 50 gallons of cold water.

To the shell particles there is now added 24 gallons of water, 23 pounds of trisodium phosphate, 1 pound of ammonium chloride and 2 pounds of sodium carbonate and 50 cc. of a fluorescene dye solution (made by dissolving 4 g.

25 of fluorescene dye in 400 cc. of water). The shell mass is allowed to remain in this solution for 20 hours at room temperature and then the liquor is poured off and the resulting exfoliated crystals 30 are washed until the powdered fragments and chemicals are removed. Thereafter the crystals are dried at 200° F. The crystals so produced have a silvery opaque background with a sparkling iridescent coating.

35 *Example 3*

75 pounds of clean Kapiz shells are crushed or ground to particles having dimensions of between  $\frac{1}{8}$  and  $\frac{1}{2}$ . The ground shell particles

40 are submerged in 17½ gallons of water to which 750 g. of sodium hydroxide is added to produce a solution having a normality of N/3 to N/4. The shells are allowed to remain in this solution for 1 hour and are stirred several times during that 45 hour. The solution is then removed and the particles are washed three times with water. The crystals of the shell particles are partially exfoliated at this point in the process.

The shell particles retain a considerable

50 amount of the wash water and to the water containing shell particles 3½ gallons of a 15% aqueous solution of gaseous chlorine and enough water to raise the level of the solution to the original amount of 17½ gallons are added (about 55 9 gallons of water are usually required). The shell particles are permitted to soak in this solution for 1 hour and then the solution is drained off and the particles are washed three times with cold water.

60 To the shell particles and entrained wash water, 5 gallons of a solution containing  $\frac{1}{2}$  lb. of sodium carbonate and 12 lbs. of trisodium phosphate are added. The shell particles are left in this solution, with occasional gentle stirring for 65 15 hours. This completes the exfoliation of the crystals. The resultant crystals are washed with cold water and dried at 200° F.

*Example 4*

70 Occasionally it is necessary to treat shells which are very dirty and the following procedure is recommended. The shells are ground as to a particle size the dimensions of which are  $\frac{1}{8}$  to  $\frac{1}{2}$ . The crushed or ground shell particles are 75 placed in a cylindrically shaped sieve the open-

ings of which are slightly less than the smallest dimension of the particles. This sieve containing the particles is rotated in a hot liquid bath containing a detergent. For example, a bath containing 13 lbs. of trisodium phosphate and 1 lb. of soap powder at 200° F. is satisfactory. The shell particles are rotated in the sieve until cleaned which may take as long as 1-2 hours depending on the condition of the shells. This treatment, in addition to washing out the dirt and small shell fragments and dust, starts the exfoliation process. The product is finally rinsed with water.

The shell particles (containing entrained water) are then treated with 8½ gallons of a solution containing 13 lbs. of trisodium phosphate, ½ lb. of sodium carbonate and 165 fluid oz. of a 30% hydrogen peroxide solution are added to the treating liquor. This treatment is continued for 2 hours.

The resultant shell particles are then washed and submerged in water to which hydrochloric acid is added in sufficient amount to make about a 3% solution. This treatment is continued for 20 minutes and the product is immediately washed with at least 3 rinses of water. This treatment removes the backs of the shells and the surface layers of crystals which might have been damaged by the hot washing treatment.

This product which is almost completely exfoliated is further treated for about one hour with an aqueous solution containing about 3½% of chlorine gas to further bring out the silvery luster of the crystals.

The crystals are washed and the exfoliation is completed in an aqueous solution containing 10-12% of trisodium phosphate and ½% of sodium carbonate. This final mix is gently stirred occasionally to facilitate separation of the crystals. The resultant crystals are washed, dried, sieved to remove small particles and packed.

The crystals produced by the above processes are substantially flat two dimensional crystals having one narrow dimension of about  $\frac{1}{16}$ " to  $\frac{1}{8}$ " and one long dimension of about  $\frac{1}{8}$ " to  $\frac{1}{4}$ ". The crystals have a silvery iridescent luster which is even superior to that of the crystals when seen in the original shell. When fluorescene dye is included in the treating solution the crystals also have a pinkish case or a bluish or greenish case when umbelliferone is included in the treating liquid.

I claim:

1. A process of obtaining silvery, iridescent crystal platelets from fresh water and marine shells comprising the steps of dividing the shells into small fragments, treating the shell fragments with an aqueous alkaline solution containing an alkali phosphate compound and having a pH of 10-13 at temperatures of less than 60

70° C. to exfoliate the crystal platelets.

2. A process of obtaining silvery, iridescent crystal platelets from fresh water and marine shells comprising the steps of dividing the shells

into small fragments, treating the shell fragment with an aqueous alkaline solution containing an alkali phosphate compound and having a pH of 10-13 at temperatures of less than 70° C. 5 discontinuing the treatment before the crystal platelets are completely exfoliated, treating the partially exfoliated crystal platelets with an aqueous solution consisting essentially of water and an oxidizing gas, and completing the exfoliation by treatment with an aqueous alkaline solution containing an alkali phosphate compound and having a pH of 10-13 at temperatures of less than 70° C.

3. A process of obtaining silvery, iridescent crystal platelets from fresh water and marine shells comprising the steps of dividing the shells into small fragments, removing the back portions of the shells, treating the shell fragments with an aqueous alkaline solution containing an alkali phosphate compound and having a pH of 10-13 at room temperature discontinuing the treatment before the crystal platelets are completely exfoliated, treating the partially exfoliated crystal platelets with a solution containing 20 an oxidizing gas, washing the resultant mass, and completing the exfoliation by treatment with an aqueous alkaline solution containing a fluorescene dye and an alkali phosphate compound and having a pH of 10-13 at room temperature.

4. A process of obtaining silvery, iridescent crystal platelets from fresh water and marine shells comprising the steps of dividing the shells into small fragments, treating the shell fragments at room temperature with an alkali hydroxide solution of less than normal strength to start exfoliation of the crystal platelets, washing the resultant mass, treating the partially exfoliated crystal platelets with an aqueous solution consisting essentially of water and an oxidizing gas, washing the resultant mass, and completing the exfoliation by treatment with an aqueous alkaline solution containing an alkali phosphate compound and having a pH of 10-13 at temperatures of less than 70° C.

5. A process of obtaining silvery, iridescent crystal platelets from fresh water and marine shells comprising the steps of dividing the shells into small fragments, treating the shell fragments with an aqueous alkaline solution containing a fluorescent dye, an alkali phosphate compound and having a pH of 10-13 at temperatures of less than 70° C. to exfoliate the crystal platelets.

JOSEPH H. HOOTON.

#### REFERENCES CITED

The following references are of record in the file of this patent:

#### UNITED STATES PATENTS

| Number    | Name         | Date           |
|-----------|--------------|----------------|
| 1,570,183 | Rauschenberg | Jan. 19, 1926  |
| 2,172,369 | Eolis        | Sept. 12, 1939 |